

Patented Nov. 30, 1943

2,335,739

# UNITED STATES PATENT OFFICE

2,335,739

## COATED FABRIC

Merle H. Chamberlin, Newburgh, N. Y., assignor  
to E. I. du Pont de Nemours & Company, Wil-  
mington, Del., a corporation of Delaware

No Drawing. Application January 31, 1942,  
Serial No. 428,979

16 Claims.

(Cl. 117—86)

This invention relates to nitrocellulose coated sheets, including non-woven paper sheets and woven fabric sheets, which contain a material which will discolor nitrocellulose.

In my copending application Ser. No. 416,601, filed October 25, 1941, there is disclosed and claimed a stain resistant nitrocellulose coated fabric which is surfaced with a layer of either cellulose acetobutyrate or cellulose acetopropionate. This material is resistant to staining by colored cosmetics, foodstuffs, etc.

In the coated fabric industry the base fabric, usually cloth or paper, is often dyed a color approximately the color of the coating which is to be subsequently applied. The dyes employed are water-soluble and do not bleed when contacted with organic solvents which are employed in cellulose derivative compositions. When a paper base is made from reclaimed rags which are usually dyed, occasionally small quantities of an oil or spirit soluble dye will be carried over to the paper base. When a nitrocellulose containing composition is applied over a base material containing only traces of oil or spirit soluble, the dyestuff will bleed up through the nitrocellulose coating and the dye color will appear on the surface of the coating, thus marring the appearance of the finished product. This is extremely objectionable where the nitrocellulose coating is of a shade lighter than the dyestuff color.

Also in the dyeing of fabrics with water soluble dyes to be subsequently coated with organic solutions of nitrocellulose compositions the dyes employed frequently become contaminated with traces of oil or spirit soluble dyestuffs which will remain on the fabric after dyeing and will bleed up through the nitrocellulose coating.

In the case of paper made from reclaimed dyed rags, it is not practical to extract the oil or spirit soluble dyestuffs before converting the rags into paper sheets and, therefore, such paper has not found widespread use as a base for nitrocellulose coatings. These papers have been confined to black coatings which would not show the discoloration resulting from the contaminating dyestuff.

The paper stocks suitable for coating with nitrocellulose coatings may also be impregnated with rubber compositions containing an antioxidant for the rubber. These rubber antioxidants will discolor nitrocellulose compositions, particularly the light colored compositions. Also bituminous plasticizers, such as asphalt, are sometimes used in paper stocks which are to be coated with nitrocellulose compositions. The bituminous

plasticizers will also discolor light colored nitrocellulose coatings applied over such a paper base.

This invention has as a primary object, the provision of a simple and economical method of preventing the discoloration of nitrocellulose coatings applied over a paper or fabric bases containing a material which will discolor nitrocellulose, and does not require any procedure or apparatus other than that now used in the coated fabric and paper industry. This objective, as well as other important but subsidiary objectives will become readily apparent to those skilled in the art as the description of the invention proceeds.

These objects are accomplished by applying a barrier coating of a cellulose acetopropionate or cellulose acetobutyrate directly over the fabric or paper base containing either spirit or oil soluble dyestuff, rubber antioxidant, or a bituminous plasticizer, and subsequently applying a nitrocellulose coating over the barrier coat. The barrier coating will not permit the migration of the nitrocellulose staining material up through to the nitrocellulose.

The following description of the preferred embodiment is given by the way of illustration and not limitation; it being understood that the invention is not to be limited to this preferred embodiment.

### EXAMPLE I

A woven cotton fabric running 1.32 yards per pound per 53 inch width and having a sateen weave was dyed with an oil or spirit soluble dyestuff. A plurality of coats of a cellulose acetopropionate coating of the following approximate composition was applied by means of a doctor knife.

#### Base coating composition

|                                | Per cent<br>by weight |
|--------------------------------|-----------------------|
| Cellulose acetopropionate      | 18.75                 |
| Ethyl phthalyl ethyl glycolate | 6.25                  |
| Ethyl alcohol                  | 37.50                 |
| Ethyl acetate                  | 37.50                 |

Sufficient coats of the above composition were applied to deposit 2 ounces per yard per 50 inch width of the non-volatile components. The method of preparing the above composition is well known in the art and further detailed description does not appear to be necessary. The volatile solvents were expelled between each successive coat of the composition by passing the material through a heated chamber.

The material was then given a plurality of coats of the following composition:

*Surface coating composition*

|                   | Per cent by weight |
|-------------------|--------------------|
| Cellulose nitrate | 14.10              |
| White pigment     | 14.57              |
| Castor oil        | 24.76              |
| Ethyl alcohol     | 23.28              |
| Ethyl acetate     | 23.29              |

The volatile solvents were expelled by passing the coated fabric through a heated chamber. The surface coating firmly anchored to the cellulose acetopropionate coating. Sufficient surface coating composition was applied to deposit approximately 15 ounces of non-volatile components per yard for 50 inch width. The coated fabric was next ornamented by embossing. Either the roller or plate type of embossing may be employed.

The white coating did not become discolored upon storage at 150° F. over night or upon prolonged storage for several months. A coated fabric identical to that described above, in which the barrier coat was omitted, was made as a control and the white coating became discolored by the oil soluble dyestuff when stored overnight at 150° F. and when stored at room temperature for a period of one week.

*EXAMPLE II*

The following composition has been found satisfactory as barrier coats to be applied directly over a fabric or paper base containing an oil or spirit soluble dyestuff which is subsequently over coated with conventional plasticized nitrocellulose compositions:

*Base coating composition*

|                                                       | Per cent by weight |
|-------------------------------------------------------|--------------------|
| Cellulose acetobutyrate                               | 18.75              |
| Mixture of ortho- and para-toluene ethyl sulfonamides | 6.25               |
| Ethyl alcohol                                         | 37.50              |
| Ethyl acetate                                         | 37.50              |

*EXAMPLE III*

A film deposited from the following composition is a satisfactory barrier to the passage of oil or spirit soluble dyestuff, rubber antioxidants and bituminous materials contained in paper or fabric sheet material:

*Base coating composition*

|                                                       | Per cent by weight |
|-------------------------------------------------------|--------------------|
| Cellulose acetobutyrate                               | 17.90              |
| Zinc oxide                                            | 13.84              |
| Mixture of ortho- and para-toluene ethyl sulfonamides | 6.92               |
| Ethyl alcohol                                         | 30.67              |
| Ethyl acetate                                         | 30.67              |

While in the preferred embodiment of this invention the barrier coat of cellulose acetopropionate or cellulose acetobutyrate is applied directly over the base material containing either an oil soluble dyestuff, rubber antioxidant or a bituminous material, it may be sandwiched in between two layers of cellulose nitrate coatings. This is particularly advantageous in commercial production when the cellulose nitrate coating is applied over a dyed cotton fabric or paper base in which the dye for the fabric or paper dye was unknowingly contaminated with oil soluble or spirit soluble dyestuff and was not detected until a portion of the nitrocellulose coating had been

applied. A barrier coat of either the cellulose acetopropionate or cellulose acetobutyrate composition may be applied over the discolored nitrocellulose coating and a sufficient coating of additional nitrocellulose composition applied over the intermediate barrier coat to hide discolored areas since the barrier coat is usually unpigmented and does not conceal the stained areas.

In the preferred examples the barrier coat is a mixed ester of cellulose, such as cellulose acetobutyrate and cellulose acetopropionate.

It is also to be understood if the base material containing the oil or spirit soluble dyestuff is to be coated on each side, it is necessary to apply the barrier coat on each side of the base material. Also if the sheet base material containing a nitrocellulose staining material is to be coated on one side only and to be stored for any length of time in roll form where the coating is in direct contact with the uncoated side of the base material, it is desirable to apply a barrier coat on each side of the base material in order to seal in the nitrocellulose staining material and prevent contact with the nitrocellulose coating.

While the invention has been described with respect to a specific construction of a coated fabric, it will be readily apparent to those skilled in the art that the invention can be utilized with any pyroxylin coated fabric construction or pyroxylin coated paper. There is no limitation to be placed upon the nitrocellulose composition which is applied over the barrier coat in accordance with the teachings of this invention.

The plasticizer for the cellulose acetopropionate or cellulose acetobutyrate is preferably one which does not have an affinity for the oil or spirit soluble dyestuffs, commonly used in the dyeing of fabrics or paper to form the base of pyroxylin coated sheets. Plasticizers for the cellulose acetopropionate or cellulose acetobutyrate, other than those mentioned in the examples, which have been found to be satisfactory for the purpose of this invention are triethylene glycol dihexoate, dibutyl phthalate, dibutyl tartrate, triethylene glycol dicaprylate, tricresyl phosphate, tributyl phosphate and the dibutyl ester of sebacic acid.

It has been found that the resistance of the barrier coat to the passage of the nitrocellulose staining material is in proportion to the amount of plasticizer content present. It has been discovered that if the plasticizer content of the barrier coat is increased beyond 65% of the total amount of non-volatile components of the barrier coat, that it is not sufficiently resistant to the oil or spirit soluble dyestuff.

In the preferred embodiment the nitrocellulose overcoating contains an oil or softener and a pigment. It has been found that the oil or spirit soluble dyestuffs, rubber, antioxidants, and bituminous plasticizers will disolor unpigmented, plasticized nitrocellulose films. Also these materials will disolor unpigmented, and unplasticized nitrocellulose films.

This invention will find great utility in the field of nitrocellulose coated fabrics and papers in using base materials which unknowingly become contaminated during the dyeing process with spirit or oil soluble dyestuffs which otherwise could only be used as a base for very dark or black shades. Also the invention will find great use in coating papers containing nitrocellulose discolored materials such as rubber antioxidants, and bituminous materials. Where the dyed base material is unknowingly contam-

inated with oil soluble dyestuff, it is not normally encountered until the first one or two coats of the cellulose derivative are applied at which time a layer of the barrier coat can be applied over the discolored coating and then the cellulose derivative coating applied over the barrier coat.

An advantage of this invention is that it allows the use of paper base material made from reclaimed rags which contains oil soluble dyestuffs for light colored pyroxylin coatings. A further advantage is that it permits the use of water soluble dyestuffs which have become contaminated with oil or spirit soluble dyestuff for dyeing paper or fabric sheets which are to be subsequently coated with compositions containing organic solvents in which case the oil or spirit soluble dyestuff does not bleed up to the surface of the coating.

It is apparent that many widely different embodiments of this invention may be made without departing from the spirit and scope thereof, and therefore, it is not intended to be limited except as indicated in the appended claims.

I claim:

1. A base material containing a nitrocellulose discoloring agent said base material having superposed on at least one side thereof a coating of a mixed cellulose ester of a plurality of lower aliphatic acids, said mixed ester being characterized by its resistance to coloring by said agent and an overcoating of a nitrocellulose composition, said nitrocellulose composition being characterized in that it is susceptible to coloring by said agent.

2. The product of claim 1 in which the mixed cellulose ester comprises cellulose acetopropionate.

3. The product of claim 1 in which the mixed cellulose ester is cellulose acetobutyrate.

4. A dyed fabric base material containing a nitrocellulose discoloring agent said base material having superposed on at least one side thereof a coating of a mixed cellulose ester of a plurality of lower aliphatic acids, said mixed ester being characterized by its resistance to coloring by said agent and an overcoating of a nitrocellulose composition, said nitrocellulose composition being characterized in that it is susceptible to color by said agent.

5. The product of claim 4 in which the mixed ester comprises cellulose acetopropionate.

6. The product of claim 4 in which the mixed

ester of cellulose comprises cellulose acetobutyrate.

7. A dyed paper base material containing a nitrocellulose discoloring agent having superposed on at least one side thereof a coating of mixed cellulose ester of a plurality of lower aliphatic acids, said mixed ester being characterized by its resistance to color by said agent and an overcoating of a nitrocellulose composition, said nitrocellulose composition being characterized in that it is susceptible to color by said agent.

8. The product of claim 7 in which the mixed ester of cellulose comprises cellulose acetopropionate.

9. The product of claim 7 in which the mixed ester of cellulose comprises cellulose acetobutyrate.

10. A dyed sheet base material containing a nitrocellulose discoloring agent said base material having superposed on both sides thereof a coating of a mixed cellulose ester of a plurality of lower aliphatic acids, said mixed ester being characterized by its resistance to coloring by said agent and an overcoating of a nitrocellulose composition, said nitrocellulose composition being characterized in that it is susceptible to coloring by said agent.

11. The product of claim 10 in which the mixed cellulose ester comprises cellulose acetopropionate.

12. The product of claim 10 in which the mixed cellulose ester comprises cellulose acetobutyrate.

13. A dyed sheet base material containing a nitrocellulose discoloring agent said base material having a first coating of nitrocellulose applied directly thereto, a second coating of a plasticized cellulose ester of mixed lower aliphatic acids composition superposed on the first mentioned coating, a third coating of nitrocellulose applied over said second coating, the said first and third coatings being characterized in that they are susceptible to coloring by said discoloring agent.

14. The product of claim 13 in which the mixed ester is cellulose acetopropionate.

15. The product of claim 13 in which the mixed ester is cellulose acetobutyrate.

16. The product of claim 13 in which the plasticizer in the mixed ester coat is less than 65 per cent thereof.

MERLE H. CHAMBERLIN.